

Aug. 13, 1940.

G. F. NADEAU ET AL

2,211,346

REMOVABLE COATING FOR PHOTOGRAPHIC FILM

Filed May 12, 1939

FIG. 1



FIG. 2



GALE F. NADEAU  
ALFRED D. SLACK  
INVENTOR

BY *Newton M. Lewis*  
*R. Frank Smith*  
ATTORNEYS

Patented Aug. 13, 1940

2,211,346

# UNITED STATES PATENT OFFICE

2,211,346

## REMOVABLE COATING FOR PHOTOGRAPHIC FILM

Gale F. Nadeau and Alfred D. Slack, Rochester, N. Y., assignors to Eastman Kodak Company, Rochester, N. Y., a corporation of New Jersey

Application May 12, 1939, Serial No. 273,298

11 Claims. (Cl. 95—9)

This invention relates to photographic film and particularly to film having overcoating or backing layers removable in photographic baths.

The desirability of anti-halation layers or overcoating layers for photographic films and plates is well known. It is also known that some of these materials are sometimes difficult to remove due to lack of solubility of one or more of the backing or overcoating constituents in the regular processing baths or to the actual repellancy of the aqueous solutions by one or more of the constituents of the backing or overcoating layer. An example of this is an anti-halation backing which is applied to the film base or plate as a material which swells or dissolves in regular developing solutions, followed by an overcoating of a water-insoluble dyestuff or coloring material. When immersed in the developing baths, the first applied layer is supposed to dissolve or wash away from the film or plate carrying the overcoated dye layer with it. If, however, this dye layer or the carrier itself is either slowly soluble or actually repellant to the developing solutions, removal may be either slow or incomplete, or in some extreme cases there may be no removal at all.

It is, therefore, an object of the present invention to provide novel means for backing or overcoating photographic films or plates. A further object is to provide a backing or an overcoating layer which is readily removable in photographic processing baths. A still further object is to provide a backing or overcoating layer having increased wettability by the processing solutions. A still further object is to provide a backing or overcoating layer containing a wetting agent which functions as a dispersing agent for the removed particles, so that they are dispersed in the wash water or processing baths and are not removed in large pieces.

These objects are accomplished by incorporating in or over the backings or overcoatings certain materials which greatly increase the susceptibility of the backing or overcoating to the processing solutions. A material of this type consists of the water soluble salts of esters of sulfo aliphatic dicarboxylic acids.

In the accompanying drawing, Fig. 1 is an enlarged sectional view of a film having an anti-halation backing according to our invention, and Fig. 2 is an enlarged sectional view of a photographic film having an overcoating layer according to our invention.

In the practice of our invention a suitable amount of the wetting agent is applied to the overcoating or backing layer from a solvent solution, or in the case of an anti-halation layer, it is convenient to apply it in the dye solution itself. The wetting agent may also be contained

in the backing or overcoating layer for the purpose of increasing the susceptibility of the layer to the processing baths. The amount of wetting agent used is determined by the degree of wettability desired, the compatibility of the particular wetting agent with the dye solution (in the case of an anti-halation backing), and the degree to which the given weight of wetting agent will reduce the surface tension at the interface of liquid and solid.

Specific wetting agents which we have found suitable for this purpose are the water-soluble salts of esters of sulfo aliphatic dicarboxylic acids, such as the calcium or sodium salt of diethyl sulfosuccinate, sold under the trade name Aerosol AY and the sodium salt of dioctyl sulfosuccinate, sold under the trade name Aerosol OT. These materials are sold by the American Cyanamide and Chemical Corporation.

The material to which these wetting agents are applied may consist of any substance which is water-soluble, or forms water-soluble salts in the developer, or which is susceptible to the processing baths ordinarily used in the treatment of photographic films or plates. Suitable materials are as follows: Cellulose esters containing a free carboxyl group, such as cellulose acetate phthalate, cellulose acetate succinate, or cellulose acetate maleate, the preparation of which is described in Genung U. S. Patent 2,126,460, 30 August 9, 1938; water soluble salts of these esters, such as the ammonium and the amine salts, some of which are described in Blanchard application Serial No. 222,302, filed July 30, 1938; cellulose ethers, such as ethyl cellulose phthalate, described in Genung U. S. Patent 2,126,460; polyvinyl phthalate, described in Nadeau U. S. Patent 2,131,747, October 4, 1938; polyvinyl alcohol, described in Sheppard et al., U. S. Patent 1,768,795, July 1, 1930; agar phthalate, described in Malm et al. application Serial No. 230,504, filed September 17, 1938; and others.

The following specific examples, which are illustrative only, will serve to illustrate our invention.

### Example 1

To a photographic film base before or after application of the sensitive emulsion layer, there is applied a layer of cellulose acetate phthalate 50 from organic solvents as follows:

|                             | Grams |
|-----------------------------|-------|
| Cellulose acetate phthalate | 8     |
| Acetone                     | 70 55 |
| Methyl alcohol              | 22    |

This coating is dried down to form a continuous layer on the film and is then dyed with a solution of Spirit nigrosine NB containing the sodium salt 60

of diamyl sulphosuccinate and having the following composition:

|                                       | Grams |
|---------------------------------------|-------|
| Spirit nigrosine NB                   | 5     |
| 5 Methyl alcohol                      | 83    |
| Butyl alcohol                         | 10    |
| Sodium salt of diamyl sulphosuccinate | 3     |

This dye layer is easily wetted by the processing solutions and is completely removed. The removed backing is well dispersed in the processing solutions.

*Example II*

15 A photographic emulsion layer, after drying, is coated with a protective layer of polyvinyl phthalate containing a wetting agent and having the following composition:

|                                        | Grams |
|----------------------------------------|-------|
| Polyvinyl phthalate                    | 5     |
| 20 Methyl alcohol                      | 46.5  |
| Butyl acetate                          | 46.5  |
| Sodium salt of dioctyl sulphosuccinate | 2     |

This layer is readily removable in the processing baths.

25 In the drawing accompanying this application, Fig. 1 shows a film support backed according to our invention. As shown therein, 10 is a support of glass or suitable cellulosic material, such as cellulose nitrate, cellulose acetate, cellulose acetate propionate, cellulose acetate butyrate, or of a suitable synthetic resin, such as a polyvinyl acetaldehyde acetal resin. The support carries an emulsion layer 11 and a backing layer 12 consisting of cellulose acetate phthalate. Over the backing layer 12 there is applied an anti-halation dye or pigment layer 13 containing a salt of an ester of a sulfo aliphatic dicarboxylic acid. As shown in Fig. 2, the support 10 carries the emulsion layer 11 and an overcoating layer 14 of a water-soluble or water-susceptible cellulose ester or synthetic resin containing a salt of an ester of a sulfo aliphatic dicarboxylic acid.

30 The specific wetting agents referred to above are water soluble salts of esters of sulfo aliphatic dicarboxylic acid, or more specifically, esters of aliphatic dibasic acids having the formula:



35 where R is an aliphatic carbon chain containing at least one sulfonic acid group but no other substituent, and X is a hydrogen atom or the radical of an alcohol containing not more than twelve carbon atoms or of a phenol not connected by a carbon to carbon bond to R, and at least one of which X's is such alcohol or phenol radical. These compounds and methods for preparing them are 40 described in Jaeger U. S. Patent No. 2,028,091, January 4, 1936.

45 The aliphatic dicarboxylic acids used in the preparation of these compounds may be saturated or unsaturated and may comprise, for example, 50 mono- and di-sulfosuccinic acid, sulfochlorsuccinic, sulfoadipic acid, sulfomaleic acid, sulfopyrrotartaric acid, sulfoglutamic acid, and other sulfonated dicarboxylic acids of the aliphatic series. These acids may be esterified with a number of 55 different alcohols such as methyl, ethyl, butyl, amyl, hexyl and octyl. We prefer to use alcohols of not more than twelve carbon atoms since the wetting agents prepared with higher alcohols, although being good wetting agents, do not retain 60 their water solubility. The water soluble salts of 65

these esters are formed by reacting the sulfonic acid group of the ester with various bases such as sodium hydroxide, organic amines, such as methyl amine and tetraethanolamine, as well as other alkali bases.

70 In Staud U. S. 1,954,337, April 10, 1934, there is described a photographic film having an anti-halation backing layer or an overcoating layer of the acid form of cellulose acetate phthalate containing monoacetin for the purpose of increasing permeability of the coating. We have found, however, that the materials which we propose to use are superior to those described in the Staud patent. When using the wetting agents of the present invention, the backing layer is easily and 75 readily removed and does not contaminate the developing solution or other bath in which the layer is removed. It is important, in processing photographic film, particularly motion picture film which is subjected to continuous treatment, 80 that the backing layer be removed as quickly and completely as possible. A material which makes possible this ready removal of the backing is, therefore, highly useful and is a desirable advance in the photographic art.

85 The materials and examples of the present specification are illustrative only and it is to be understood that numerous methods and ingredients may be used within the scope of the present description, and that our invention is to be 90 taken as limited only by the scope of the appended claims.

1. A sensitive photographic element comprising a superficial coating removable in photographic processing baths and in direct contact with said coating, a water soluble salt of an ester of a sulfo aliphatic dicarboxylic acid.

2. A sensitive photographic element comprising a superficial coating removable in photographic processing baths and in direct contact with said coating, a water soluble salt of an ester of an aliphatic dibasic acid having the formula



45 where R is an aliphatic carbon chain containing at least one sulfonic acid group but no other substituent, and X is selected from the group consisting of hydrogen alcohol of not more than twelve carbon atoms or phenol radicals not connected by a carbon to carbon bond to R, at least one X being such as alcohol or phenol radical.

3. A sensitive photographic element comprising a superficial coating containing as a wetting agent a water-soluble salt of an ester of a sulfo aliphatic dicarboxylic acid and readily removable in photographic processing baths.

4. A sensitive photographic element comprising a water susceptible superficial coating and over said coating a layer containing a water soluble salt of an ester of a sulfo aliphatic dicarboxylic acid, the composite coating being readily removable in photographic processing baths.

5. A sensitive photographic element comprising a water susceptible superficial coating and over said coating a dye layer containing a water soluble salt of an ester of a sulfo aliphatic dicarboxylic acid, the composite coating being readily removable in photographic processing baths.

6. A sensitive photographic element comprising a superficial coating of cellulose acetate phthalate and over said coating a layer containing a water soluble salt of an ester of a sulfo 75

aliphatic dicarboxylic acid, the composite coating being readily removable in photographic processing baths.

7. A sensitive photographic element comprising a backing layer of cellulose acetate phthalate and over said layer a dye layer containing a water soluble salt of an ester of a sulfo aliphatic dicarboxylic acid, the composite backing being readily removable in photographic processing baths.

8. A sensitive photographic element comprising a superficial coating of a water susceptible material and over said coating a layer containing the water soluble salt of a sulfosuccinic ester, the composite coating being readily removable in photographic processing baths.

9. A sensitive photographic element comprising a backing layer of a water susceptible ma-

terial and over said layer a dye layer containing the sodium salt of an ester of sulfosuccinic acid, the composite backing layer being readily removable in photographic processing baths.

10. A sensitive photographic element comprising a superficial coating of cellulose acetate phthalate and over said coating a layer containing the sodium salt of diamylsulfosuccinate, the composite coating being readily removable in photographic processing baths.

11. A sensitive photographic element comprising a backing layer of cellulose acetate phthalate and over said backing layer an anti-halation layer containing a coloring material and the sodium salt of diamylsulfosuccinate.

GALE F. NADEAU.  
ALFRED D. SLACK.